

2,916,455

## LUBRICATING OIL COMPOSITION

Allen F. Millikan, Crystal Lake, and Gifford W. Crosby, River Forest, Ill., assignors to The Pure Oil Company, Chicago, Ill., a corporation of Ohio

No Drawing. Application November 5, 1956  
Serial No. 620,198

4 Claims. (Cl. 252—46.4)

This invention relates to lubricating oils, particularly those used in the crankcases of automotive vehicle motors.

It is common practice to add to mineral lubricating oils used to lubricate internal combustion engines various additives for the purpose of imparting to the oil high detergency, high load-carrying characteristics, low wear and low corrosion qualities. Among the well-known compounds for imparting improved load-carrying and wear characteristics are the zinc alkyl thiophosphates and the alkyl, aryl and alkylaryl thiophosphites.

We have discovered that certain arsenic compounds give to a lubricant better load and wear characteristics than phosphorus compounds. The arsenic compounds of our invention, when added to mineral lubricating oil in amounts sufficient to give an arsenic content of between 0.1 and 2% by weight of the finished blend, have an unexpected effect in improving the load-carrying characteristics of the lubricating oil. The arsenic compounds of this invention belong to the class represented by the general formula



in which  $R_1$ ,  $R_2$  and  $R_3$  are selected from the group consisting of aryl, alkyl, arylalkyl and alkylaryl radicals and may be the same or different. We prefer those compounds in which  $R_1$ ,  $R_2$  and  $R_3$  are aryl or alkyl-substituted aryl groups. As examples of trithioarsenites which are suitable for the purposes of our invention may be mentioned triphenyl, tritolyl, trixyl, trimethylxenyl, triethylxenyl, and trianaphthyl trithioarsenites. Where  $R_1$ ,  $R_2$  and  $R_3$  are alkyl groups, it is preferred that they have at least 5 carbon atoms in the chain in order to impart sufficient solubility of the compound in the oil. As examples of alkyl and substituted-alkyl trithioarsenites the following may be mentioned: tri-2-ethylhexyl, triamyl, tri-2-ethylbutyl, tricyclohexyl, tribenzyl, triphenylethyl, triauryl, tristearyl and trioleyl trithioarsenites.

Trithioarsenites containing different  $R$  groups are il-

lustrated by amyl diphenyl trithioarsenite, phenyl di-(amylphenyl) trithioarsenite and hexyl cyclohexyl phenyl trithioarsenite.

In general, the trithioarsenites may be made by reacting arsenic trichloride with the thiol or thiophenol corresponding to the alkyl or aryl groups in the trithioarsenite which it is desired to make. For example, if it is desired to prepare triphenyl trithioarsenite, 49 gms. (0.45 mol) of thiophenol is dissolved in 200 ml. of absolute ethanol, 17.9 gms. (0.45 mol) of sodium hydroxide is added, and the mixture is heated to form a sodium thiophenate salt. A few milliliters of water are added to the reaction mixture to facilitate solution and reaction. When the mixture has almost completely gone into solution, there is added 30.1 gms. (0.165 mol) of arsenic trichloride, upon the addition of which there is immediately formed a white precipitate and a small amount of gas. The solid product is filtered and washed with five successive 100-milliliter portions of water to remove by-product sodium chloride. The product is then purified by recrystallization from a benzene-methanol solvent containing one part of benzene to three parts by volume of methanol. The yield before recrystallization is approximately 95% of theoretical. After recrystallization the yield is approximately 75%. The recrystallized product analyzes 19.7% arsenic and 23.3% sulfur, against theoretical values of 18.6% and 23.9%, respectively.

Preparation of trithioarsenites in which  $R_1$ ,  $R_2$  and  $R_3$  are different may be accomplished by the reaction of arsenic trichloride with mixtures of sulfhydryl compounds; or, if pure compounds are desired, alkyl or aryl chloroarsenites may be prepared as intermediates and converted to the final ester by reaction with the desired sulfhydryl compound, e.g.



The triphenyl trithioarsenite prepared as described was added in the amount of 2.1% by weight to a mineral lubricating oil composed of 94.1% by weight of neutral oil having a viscosity of 170 SUS at 100° F., 5.3% by weight of basic barium sulfonate and 0.65% by weight of sulfurized terpene. The sulfonate was added as a detergent and the sulfurized terpene as a corrosion inhibitor in order to approximate a finished motor oil suitable for internal combustion engine service. This blend was tested for load-carrying and wear-resistant characteristics and compared with similar blends in which a commercial zinc dialkyl dithiophosphate and triphenyl trithiophosphate were substituted for the triphenyl trithioarsenite. The blends were tested on the 4-Ball, E.P. and Wear machines, which are described by Larsen, Lubrication Engineering, 1, 35-43 (1945). The results of the tests are given in the following table.

Table

| Antiwear Additive                                                    | Wt. Percent Element in Additive | Wt. Percent of Additive in Blend | Wt. Percent of Element in Blend | Millimoles of Additive per 100 gr. of Blend | Load, kg. (constant starting temperatures) | Temperature, °F., 50 kg. Load | 20 kg., 1,800 r.p.m., 5 Minute Wear Test Scar Diameter, mm. |
|----------------------------------------------------------------------|---------------------------------|----------------------------------|---------------------------------|---------------------------------------------|--------------------------------------------|-------------------------------|-------------------------------------------------------------|
| None                                                                 |                                 |                                  |                                 |                                             | 60                                         | 200                           | 0.38                                                        |
| Commercial zinc dialkyl dithiophosphate, Zn (SP(S)(OR)) <sub>2</sub> | 7.3(P)                          | 2.6                              | 0.19                            | 6.1                                         | 100                                        | 300                           | 0.27                                                        |
| Triphenyl trithioarsenite, As(SO <sub>2</sub> H) <sub>3</sub>        | 19.7(AS)                        | 2.1                              | 0.41                            | 5.5                                         | 110                                        | 400                           | 0.30                                                        |
| Triphenyl trithiophosphate                                           | 8.7(P)                          | 2.0                              | 0.17                            | 5.5                                         | 90                                         | 250                           | 0.29                                                        |

By examining the foregoing table it will be evident that not only did the triphenyl trithioarsenite exceed the triphenyl trithiophosphite and the zinc dialkyl dithiophosphate in the high load-carrying test, but it also was able to carry a load at a much higher temperature without causing excessive wear. In the 5 minute wear test, which is a light-load wear test, there is substantially no difference between the trithioarsenite and the trithiophosphite, although both were superior to the oil containing neither of these additives.

The ability of compounds of elements of group VB of the periodic table to improve the load-carrying ability of lubricating oils cannot be predicted. In a series of tests on similar organo-phosphorus, -arsenic, -antimony and -bismuth compounds in mineral lube oil containing basic barium sulfonate and sulfurized terpene, the phosphorus, arsenic and antimony compounds all produced low wear rates, but the bismuth compound brought about an increase in wear rate. In another series of tests in neutral oil blends, the phosphorus- or arsenic-containing additives showed low wear rates, but the antimony compound showed a high wear rate. In the tests reported in the table, although the thiophosphite ester allowed a small increase in temperature for low wear operation with a standard load, the trithioarsenite ester brought about a very marked increase in allowable operating temperature, namely, from 200 to 400° F.

Although the test data were determined on a specific trithioarsenite, namely, the triphenyl trithioarsenite, it is to be understood that trithioarsenite esters in general have the ability to unexpectedly improve the load-carrying characteristics and the wear rate at high temperatures

of mineral lubricating oils and that this characteristic is particularly marked in the triaryl and alkyl-substituted triaryl esters.

We claim as our invention:

- 5 1. A lubricant consisting essentially of mineral lubricating oil and a small amount, sufficient to enhance the load-carrying and wear-resistant properties of the oil, of at least one compound corresponding to the formula:

10



where  $R_1$ ,  $R_2$  and  $R_3$  may be a radical containing 5 to 18 carbon atoms selected from the group consisting of

15 alkyl, aryl, arylalkyl and alkylaryl.

2. A lubricant in accordance with claim 1 in which the arsenic compound is present in an amount sufficient to produce an arsenic concentration of 0.1 to 2%.

3. A lubricant in accordance with claim 2 in which the compound is a triaryl trithioarsenite.

20 4. A lubricant in accordance with claim 2 in which the compound is triphenyl trithioarsenite.

#### References Cited in the file of this patent

#### UNITED STATES PATENTS

|           |              |                |
|-----------|--------------|----------------|
| 2,214,444 | Varteressian | Sept. 10, 1940 |
| 2,346,155 | Denison      | Apr. 11, 1944  |
| 2,346,156 | Farrington   | Apr. 11, 1944  |
| 2,354,536 | Nelson       | July 25, 1944  |
| 2,768,192 | McLeod       | Oct. 23, 1956  |